

Sept. 18, 1951

F. E. LATHE

2,568,237

BATCH FOR REFRACTORY MASSES AND METHOD OF CONSOLIDATING

Filed Aug. 3, 1946

4 Sheets-Sheet 1



Fig. 1.

Inventor:  
Frank E. Lathe

By Alex. E. MacRae  
Attorney.

Sept. 18, 1951

F. E. LATHE

2,568,237

## BATCH FOR REFRACTORY MASSES AND METHOD OF CONSOLIDATING

Filed Aug. 3, 1946

4 Sheets-Sheet 2



*Inventor:*

frank E. Lathe

By Alex. E. MacRae  
~~Attorney~~

Attorney.

Sept. 18, 1951

F. E. LATHE

2,568,237

BATCH FOR REFRACTORY MASSES AND METHOD OF CONSOLIDATING

Filed Aug. 3, 1946

4 Sheets-Sheet 3



Inventor:  
Frank E. Lathe  
By Alex. E. Mae Rae  
Attorney.

Sept. 18, 1951

F. E. LATHE

2,568,237

BATCH FOR REFRACTORY MASSES AND METHOD OF CONSOLIDATING

Filed Aug. 3, 1946

4 Sheets-Sheet 4



Inventor:  
Frank E. Lathe  
By Alex. E. Mac Rae  
Attorney.

## UNITED STATES PATENT OFFICE

2,568,237

BATCH FOR REFRACTORY MASSES AND  
METHOD OF CONSOLIDATING

Frank Eugene Lathe, Ottawa, Ontario, Canada,  
assignor to Canadian Refractories Limited,  
Montreal, Quebec, Canada, a corporation of  
Canada

Application August 3, 1946, Serial No. 688,264  
In Canada July 16, 1946

7 Claims. (Cl. 106—57)

1

This invention relates to the bonding of refractory materials, and in particular to a method of consolidating granular particles of refractory character, at a relatively low temperature, into highly refractory masses and shapes.

In the industrial application of refractories—as, for example, in forming furnace bottoms and in fettling open hearth and electric steel furnace banks—it is highly advantageous to use materials which will "set" or be well consolidated, at a relatively low temperature. This will obviate the necessity of driving a furnace so hard as to damage the superstructure by partial fusion of the brickwork, which is a frequent result when material, too refractory in character, is to be consolidated in the furnace lining. By reducing the maximum temperature required, and shortening the period of burning-in the bottom, important economies in both fuel and labour can be effected. By producing a more monolithic bottom, the absorption of steel and slag will be reduced, and the useful life of the refractory will be increased.

On the other hand, it is obviously important to have furnace linings made of materials sufficiently refractory that they will not fail at the highest working temperature. With the development for furnace superstructures of materials substantially more refractory than have previously been used, and the higher operating temperatures adopted as a result, the danger of breakouts and other types of hearth failure has been increased. This continued trend towards higher temperatures emphasizes the need for improved hearth refractories.

It will be seen that these two desiderata in the properties of refractories—consolidation at low temperature and resistance to failure at high temperature—are diametrically opposed. It is not too much to say that for the past twenty-five years a major objective of research on refractories has been to devise ways and means of overcoming these defects. Much ingenuity has been shown in effecting compromises between the two objectives.

In the older practice, when it was desired to make a "permanent" hearth from Austrian magnesite or other form of highly refractory periclase clinker (which cannot be burned to a monolithic mass at any permissible or readily attainable temperature), it was customary to mix with the clinker some 20–25% of slag, the purpose of which was to melt at a relatively low temperature and thus act as a bond for the more refractory particles of periclase. However, the ultimate product was

2

at best a mixture of the two materials used, and the slag matrix remained as a weak component for an indefinite period, being subject to melting at maximum operating temperatures, to chemical attack by the constituents of the furnace charge, and to physical replacement in the bottom by molten steel. Such practice, while still followed to some extent, has been largely superseded by more modern methods.

10 A major improvement was effected by the development of "magnesite" clinkers containing, as essential constituents of the clinker particles, a sufficient proportion of compounds of lower refractoriness, such as calcium ferrites and aluminates, to constitute a self-bonding material. 15 These have been called thermoplastic hearth refractories. McAnally (U. S. 1,305,475) used in his clinker 16–18% of lime and 8.0–8.5% of iron oxide plus alumina. His product could be sintered to a monolithic mass without the addition of slag, and has been widely imitated, but in his method improved setting was secured at the expense of ultimate refractoriness, since any fluxes introduced become a permanent part of the hearth, and are converted to the liquid condition whenever the temperature rises sufficiently high. 20 Using the same principle, McCaughey and Lee (U. S. 1,965,605) introduced similar proportions of calcium ferrites and aluminates into a clinker of higher magnesia content. Seaton and Hartzell (U. S. 2,218,485) used two different magnesian refractories, of such composition and in such proportions that, by their reaction with one another, dicalcium silicate, tricalcium aluminate and calcium ferrite were said to be formed. The addition 25 of slag to bond such refractories was recognized as desirable, and in fact was claimed. Later (U. S. 2,238,428), these investigators produced a refractory containing a minor proportion of monticellite ( $\text{CaO} \cdot \text{MgO} \cdot \text{SiO}_2$ ), and then converted the latter to dicalcium silicate ( $2\text{CaO} \cdot \text{SiO}_2$ ) by heating the refractory with a lime-bearing material. 30 Lee (U. S. 2,292,644) similarly improved the refractoriness of a material containing merwinite ( $3\text{CaO} \cdot \text{MgO} \cdot 2\text{SiO}_2$ ) by adding lime and heating 35 to convert at least a part of the merwinite to dicalcium silicate. Lee objected to the presence in the primary refractory of monticellite, which, he said, lowered the refractoriness too much.

40 In summary, it has previously been proposed to make refractories which would set at attainable temperatures by (1) using in furnace linings mixtures of slag and refractories high in magnesia, (2) introducing calcium ferrite and aluminate into magnesian clinkers, (3) combining a

magnesian refractory containing a little monticellite (together with iron oxide and alumina) with a material sufficiently high in lime to convert the monticellite to dicalcium silicate and periclase, and (4) making a basic refractory containing merwinite and converting at least a part of this to dicalcium silicate and periclase by firing with calcareous material.

Recently, a different method of attack on the problem has been made by the introduction of chemical bonds, such as sodium silicate, into masses of refractory clinker that are rammed into place, and thereby becomes unnecessary to give the material a prolonged heat treatment at high temperature in order to form a working bottom. This development has proved of great importance in saving time and thereby increasing plant capacity, but it has not overcome the difficulty involved in the introduction of constituents of low melting-point, and refractories of this type have been too expensive for general use in maintaining furnace banks.

For the latter purpose, so-called double-burned dolomite, containing a considerable proportion of iron oxide, has been extensively used, along with raw and calcined dolomite, but these materials afford only temporary protection to furnace banks, and their chief merit is in fact their cheapness.

In no case, it must be emphasized, do these proposals overcome both of the major difficulties set out above, and at best they constitute only various degrees of compromise. Some methods do not sufficiently lower the setting temperature to effect major economies in burning-in the original hearths or in fettling furnace banks; some permanently lower the refractoriness of the furnace materials to such a degree that subsequent service is impaired. In spite of their individual advantages, the problem remains essentially the same—that of developing a material which will set rapidly at easily attainable temperatures, and which will nevertheless have sufficient ultimate refractoriness to permit raising the operating temperature to a point well above that now used. Heretofore, no such material had been produced.

In the accompanying drawings are shown melting-point diagrams of actual or hypothetical starting materials of the character herein described to facilitate a ready understanding of the invention. The temperatures given herein are in general either those compiled by Sosman and Andersen, as given on U. S. Steel Corporation Plates 1-4 Composition - Temperature Phase Equilibrium Diagrams of the Refractory Oxides, dated October 1933, or those given in comprehensive reviews by Hall and Insley. Degrees centigrade are used throughout.

In accordance with the present invention an entirely new approach to the problem has therefore been made and, as will be seen below, it has been found that both difficulties can be overcome by simple and highly economical means. Not only is the consolidation of highly refractory particles brought about at a substantially lower temperature than has heretofore been possible without the introduction of alkali metal compounds, but the ultimate refractoriness of the furnace lining or refractory shapes is at the same time substantially enhanced.

In order to accomplish these desirable ends, it is essential to select particular starting materials. These include a considerable variety of cheap and common minerals and mineral products, but only those combinations may be used which belong to

5 a very specific type. This acceptable type is invariably characterized by (1) reaction between the starting materials, under suitable conditions, to form a definite chemical compound of high refractoriness, and (2) the formation between this chemical compound and one of the starting materials—but not the other—of a product (usually of eutectic character) which substantially or completely melts to a liquid condition at the low temperature desired. That is, the temperature of liquid formation between the compound and one starting material must always be much below that of any eutectic or other liquid which may be formed between the compound and the second starting material, and obviously far lower than the melting-point of the compound itself.

These conditions are most clearly expressed in the form shown in Fig. 1, which is a hypothetical melting-point diagram of two starting materials, A and B, of the type described, and having melting-points  $T_1$  and  $T_2$ , respectively. In order to make the illustration wholly general in character, the basic temperature is taken as  $T^\circ$ . As shown, 62% of starting material A reacts with 38% of starting material B to form the compound  $A_xB_y$ , having a melting-point  $T_3$  of approximately  $T+1400^\circ$ . This compound in turn forms with B a eutectic  $E_1$ , with a melting-point  $T_4$  of  $T+300^\circ$  and a composition of 25% A and 75% B. With A,  $A_xB_y$  forms a eutectic  $E_2$  containing 70% A and 30% B, and having a melting-point  $T_5$  of  $T+1300^\circ$ . The broken line indicates that eutectic formation between  $A_xB_y$  and A is not essential; in case of a compound having an incongruent melting-point, the temperature of complete fusion rises continuously from  $T_4$  to  $T_1$ , with marked change in rate at R, which is technically known as the reaction point. The above-stated rule nevertheless applies, for  $A_xB_y$  still forms a low-melting product with B but not with A. This distinction is fundamental.

Referring again to Fig. 1, and omitting consideration of the broken line, which applies to only a few cases, it may be pointed out that the curve is the locus of the temperature of complete fusion for every combination of A and B. Above the line, at any composition whatever, the melt is entirely liquid. At the five compositions corresponding to A,  $E_2$ ,  $A_xB_y$ ,  $E_1$  and B there are definite melting-points, these being  $T_1$ ,  $T_5$ ,  $T_3$ ,  $T_4$ , and  $T_2$ , respectively. At all other compositions, freezing and melting occur over a range of temperature. For example, at a composition of 50% each of A and B, freezing of the wholly molten material begins at about  $T+1180^\circ$ , when the compound  $A_xB_y$  begins to separate as a solid. This of course changes the composition of the remaining liquid, and with a continued drop in temperature more of  $A_xB_y$  separates until the final liquid reaches the composition  $E_1$ , at a temperature  $T_4$ , when it all solidifies. Similarly, if a melt of composition represented by 80% A and 20% B be cooled from  $T+2000^\circ$ , for example, no solid forms until a temperature of about  $T+1530$  is reached, when A begins to separate, again with a change in liquid composition. With further cooling, more A separates until the liquid composition  $E_2$  is reached, at a temperature  $T_5$ , when complete solidification again results before there can be any further temperature drop.

From this discussion it will be obvious that the hatched areas in the chart represent compositions which are completely solid at the temperatures shown. Similarly, clear areas, above the

curves, are those of complete liquidity, while stippled areas represent conditions of composition and temperature in which liquid and solid (having different compositions) co-exist in equilibrium. All of this is well known to students of phase equilibrium diagrams, but is mentioned here in order to clarify the subsequent discussion.

The actual procedure to be followed in carrying out the principles of this invention may now be explained for the general case of two starting materials, A and B, again with reference to Fig. 1. Both, it will be observed, are of a refractory character, although it may be assumed that the more refractory material A is to be the major constituent of the final product. First, one takes 25% of A and 75% of B (corresponding to the composition of  $E_1$ ), melts the mixture at a temperature  $T_4$  ( $T+300$ ) and allows the product to solidify. Twenty parts of the crushed product (containing five parts of A and fifteen of B) are then mixed with eighty parts of A, of any suitable grain size, and the mixture is formed into the desired shape, rammed into a furnace to form a permanent hearth, or thrown as fettling material into a hot furnace. When the temperature of the mass is raised to  $T+300$ , the 20% of constituent  $E_1$  melts, and this sets or consolidates the whole mass of A particles. As the temperature is raised towards the normal operating temperature of the furnace, however, the liquid formed reacts with the solid particles of A to form  $A_xB_y$ . By the time the reaction is complete all liquid has disappeared and, because the mass contains a greater proportion of A than that corresponding to  $A_xB_y$ , no more liquid can form until  $T+1300$  (the melting-point of  $E_2$ ) is reached. Mineralogically, the final refractory consists entirely of A and  $A_xB_y$  in equilibrium with each other; the relative amounts will depend always of course, upon the proportions of the starting materials used.

In this case, it is evident that a very striking and important result has been brought about. By using two refractory starting materials of the specified type, it has been possible through the application of the present invention to consolidate highly refractory particles of A into a furnace hearth (mass or shape) at a temperature 1000 degrees below that at which initial liquid formation can subsequently occur, and in fact 900 degrees below the melting-point of either starting material.

It is important to observe that the two starting materials do not have to be taken in the exact proportions corresponding to the eutectic  $E_1$  in order to form a low-melting product. In the case of these two starting materials, a large proportion of liquid will be formed at  $T_4$  even though the composition may be varied, for example, anywhere from 40% A and 60% B to 12% A and 88% B. At the former composition, 59.5% of liquid  $E_1$  will form at  $T_4$  with 40.5% of solid  $A_xB_y$ , and complete liquidity will result at about  $T+900$ , while at the latter composition there will be 48% of liquid  $E_1$  at  $T_4$  with 52% of solid B, and the whole mass will again be molten at  $T+900$ . (The proportion of solid and liquid may be determined by measurement from the chart, or may be calculated algebraically; both methods are well known to students of phase equilibrium diagrams.)

It may also be observed that when the proportion of starting material B is greater than 38%, some liquid will always be formed at  $T_4$ , the melting-point of the eutectic  $E_1$ , whereas with

38% or less there will be no liquid under the temperature  $T_5$ , which is the melting-point of  $E_2$ . At 38% of B there will, of course, be none of either eutectic present, and no liquid will be formed below  $T_3$ , at which temperature the compound  $A_xB_y$  melts completely. The low-melting constituent used in practice must therefore have a greater proportion of starting material B than is present in  $A_xB_y$ , and the only precaution necessary to eliminate all low-melting liquid in the ultimate product is to use enough of A in the final mixture to form the compound  $A_xB_y$  with all of the starting material B present. It may be advantageous to use a much greater proportion of A if this particular refractory is superior to  $A_xB_y$  in the properties desired in the ultimate product.

In all the above discussion consideration has been given to the general case. Attention will now be called to combinations of actual starting materials of the same type. These cases are not all equally simple, but the essential features enumerated above are identical, and such differences as occur will be explained.

One of the most interesting cases is that of lime and silica (Fig. 2), which have melting-points of 2570 and 1728°, respectively. They form a highly refractory compound, dicalcium silicate ( $2CaO \cdot SiO_2$ ), which has a melting-point of 2130°. The lowest-melting eutectic contains 36% lime and 64% silica, and this melts at 1438, whereas the eutectic between dicalcium silicate and lime has a melting-point of 2065, 627 degrees higher, and no liquid can form below this temperature if the proportion of lime to silica is that of dicalcium silicate or greater. This case differs from the one described in Fig. 1 in that there is an intermediate compound, calcium metasilicate



having a melting-point of 1544° and, strictly speaking, it is this compound which forms two low-melting eutectics. Both of these eutectics, it may be observed, have melting-points about 200 degrees below the ordinary operating temperature of an open hearth or electric steel furnace, whereas the refractory eutectic between dicalcium silicate and lime melts at a temperature far above any thing used in furnaces of these types.

Of the same type is the melting-point diagram of magnesia and silica, as shown in Fig. 3. The compound between these two starting materials is the orthosilicate ( $2MgO \cdot SiO_2$ ) forsterite, which has a melting-point of 1910°. The low-melting eutectic melts at 1547° and the high-melting eutectic—between forsterite and magnesia—at 1870, 323 degrees higher. The latter temperature is at least 200 degrees above ordinary open hearth temperatures, and if the magnesia content be high the percentage of liquid formed even at that temperature is relatively small. Magnesia itself has a melting-point of 2800°. This case differs from that of lime and silica in that the metasilicate has an incongruent melting-point, but this is of no practical importance, and the resemblance is otherwise quite close.

Of some interest (but not illustrated) is the system lime-alumina. Both of these oxides are highly refractory. In this case there are several compounds, of which the most refractory is  $3CaO \cdot 5Al_2O_3$ , having a melting-point of 1735 and forming with alumina a refractory eutectic melting at 1715°. There are two low-melting eutectics, that between  $3CaO \cdot Al_2O_3$  and  $5CaO \cdot 3Al_2O_3$ , melting at 1397, and that between  $5CaO \cdot 3Al_2O_3$  and

$\text{Ca}_2\text{Al}_2\text{O}_5$ , melting at 1402°. Both, or any composition of lime and alumina containing between 45 and 60% alumina, can be used satisfactorily to bond particles of refractory alumina, and provided that the proportion of alumina in the mixture be at least that in  $3\text{CaO} \cdot 5\text{Al}_2\text{O}_5$  (75.2%), no liquid can form below 1715°.

Of substantially different form, but corresponding somewhat to that of the dotted line of Fig. 1, is Fig. 4, of alumina and silica. In this case the low-melting eutectic is exceptional in that it contains about 94% of one starting material—in this case silica. Its melting-point is 1550°. The refractory compound  $3\text{Al}_2\text{O}_5 \cdot 2\text{SiO}_2$  (mullite) has an incongruent melting-point of 1830°, and forms no eutectic with alumina, so that when the low-melting eutectic is eliminated the temperature of initial liquid formation is raised by 280 degrees. All that is necessary to eliminate the low-melting liquid is to increase the overall alumina content to 72% or higher, the composition corresponding to mullite. The principle is identical with that previously set out.

A striking example is that of Fig. 5, of baryta and zirconia, but this system has not been reported in complete detail. The refractory compound barium-zirconate ( $\text{BaO} \cdot \text{ZrO}_2$ ) has a melting-point of at least 2600°, while the low-melting eutectic containing about 10% (molecular) of zirconia melts at approximately 1300°. The eutectic between barium zirconate and zirconia has a melting-point of approximately 2050, or higher, by 750 degrees.

All of the above examples, both theoretical and practical, have dealt with binary systems, the two starting materials being in all cases refractory oxides. Exactly the same principle, however, may be applied when there are three starting materials, or, to express the idea differently, when one of the starting materials consists of two oxides, which may or may not exist in chemical combination with each other.

Fig. 6 illustrates the general case of three refractory oxides, A, B, and C, having melting-points of about  $T+1900$ ,  $T+1600$ , and  $T+2000$ ° respectively. As before, there is a refractory compound  $\text{A}_x\text{B}_y$ , which forms a low-melting eutectic with B, or with B and C, and a high-melting eutectic with A, or with A and C. In the presence of starting material C the melting-points of both binary eutectics are lowered somewhat, but it still holds that the lowest-melting eutectic between A, B and C (or, strictly speaking, between  $\text{A}_x\text{B}_y$ , B and C) can be completely eliminated by heating it with at least enough of A to convert all of B to  $\text{A}_x\text{B}_y$ . This case has been oversimplified, in order to illustrate the point, by assuming that B and C are taken in constant proportions, with reference to each other, and that the two eutectics lie on the same straight line drawn through A to (B+C). This constant proportion of two starting materials, however, is a frequent commercial condition.

The pseudobinary melting-point diagram of A and (B+C), as derived from Fig. 6 is shown in Fig. 7, and it will be observed that it has a form very similar to that of Fig. 1. In this case the compound  $\text{A}_x\text{B}_y$  (as modified by the presence of about 10% of C) melts at about  $T+1400$ , one eutectic melts at  $T+300$  and the other at  $T+1200$ °. The principle already explained for Fig. 1 can be applied in exactly the same way in this case by preforming a low-melting eutectic of A, B, and C, and using this to set or consolidate, at a low temperature, highly refractory particles of A.

The temperature of initial liquid formation is thereby raised 900 degrees.

To pass again from the general to the specific, one may take, as in Fig. 8, the two starting materials silica and calcined dolomite, and plot the melting-point curve as a pseudobinary system. It is seen that the compound dicalcium silicate can co-exist with periclase. Complete fusion of a low-melting product, with a silica content of about 50%, can be made to occur at 1358, but, by burning it with sufficient lime to form dicalcium silicate with all of the silica thus introduced, the temperature of initial liquid formation can be raised by 622 degrees to 1980°. This particular chart does not show a high-melting eutectic, since the pseudobinary line does not pass through it, but such a eutectic nevertheless exists, with 1980 as its approximate melting-point.

Another case of a pseudobinary is that of Fig. 9, which illustrates the same principle when applied to magnesia, and a hypothetical clay containing silica and alumina in the proportions 70 to 30. This case is of special interest in that the magnesia decomposes the clay to form not one, but two, compounds, these being forsterite and spinel ( $\text{MgO} \cdot \text{Al}_2\text{O}_3$ ), which can co-exist in equilibrium. Liquid formation can take place at a temperature as low as 1347, with complete fusion at 1362, yet all low-melting liquids can be eliminated by heating with sufficient magnesia, the temperature of initial liquid formation then becoming about 1700°, or substantially the melting-point of pure silica. In products of high magnesia content, relatively little liquid will be formed, even at this temperature.

It is obvious that, if a low-melting rock or mineral of suitable composition be available, this may be used in place of an artificial product made by fusion of the two starting materials. For example, both diopside ( $\text{CaO} \cdot \text{MgO} \cdot 2\text{SiO}_2$ ) and tremolite ( $\text{CaO} \cdot 3\text{MgO} \cdot 4\text{SiO}_2$ ) melt below 1400, wollastonite ( $\text{CaO} \cdot \text{SiO}_2$ ) at 1544, cordierite ( $2\text{MgO} \cdot 2\text{Al}_2\text{O}_3 \cdot 5\text{SiO}_2$ ) at 1530 and enstatite ( $\text{MgO} \cdot \text{SiO}_2$ ) at 1547°. These minerals are of common occurrence in pyroxenites, amphibolites and related rocks.

Now that the principle of the invention has been fully explained and illustrated, it may be accurately redefined as a method of consolidating refractory granular materials, at a relatively low temperature, into masses or shapes of a highly refractory character, which comprises (a) the selection of two refractory materials of the type illustrated in Fig. 1 (or of more than two, as illustrated in Fig. 7), characterized by the formation between them of at least one highly refractory chemical compound, which compound unites or reacts with the first but not with the second starting material to form an intermediate compound, eutectic or other product of relatively low refractoriness, (b) forming by any convenient means said intermediate compound, eutectic, or other product of low refractoriness, or utilizing a natural mineral or rock of similar chemical composition and properties, (c) using said intermediate product of low refractoriness, while in a molten condition but at a relatively low temperature, to consolidate particles of the second refractory starting material into masses or shapes, and (d) converting said masses or shapes by the application of heat into highly refractory, ceramicly bonded bodies through the substantial elimination of the said intermediate prod-

uct of low refractoriness by means of its reaction with the second refractory starting material.

The starting materials must always be of the specific type described above, but it is not essential that, as taken for commercial use, they be in the particular form mentioned. For example, lime and magnesia have been given as starting materials, whereas in practice it may be more convenient to use limestone, magnesite, brucite, or dolomite, all of which on the application of heat are readily converted into the corresponding oxide or oxides. So also one may use diaspore ( $\text{Al}_2\text{O}_3 \cdot \text{H}_2\text{O}$ ) as a source of alumina, and barite ( $\text{BaSO}_4$ ) of barium oxide, and as sources of more than one oxide such minerals as wollastonite, serpentine ( $3\text{MgO} \cdot 2\text{SiO}_2 \cdot 2\text{H}_2\text{O}$ ), and kaolinite ( $\text{Al}_2\text{O}_3 \cdot 2\text{SiO}_2 \cdot 2\text{H}_2\text{O}$ ). In every case, however, the combination of oxides chosen must be such that they fall into the particular type described.

There may also be used as a major starting material a clinker containing magnesia associated with more lime than that necessary to form calcium silicate with all the silica present in it. In such a case, the magnesia is substantially inert and the excess of lime acts as one starting material, while the other is siliceous, like serpentine, diopside, wollastonite or quartzite.

As already intimated, the initial product of relatively low refractoriness need not be a true eutectic between  $\text{A}_x\text{B}_y$  and the first starting material. For some applications a low-melting compound such as pseudowollastonite (melting-point 1544) or  $5\text{CaO} \cdot 3\text{Al}_2\text{O}_3$  (melting point 1458) may be satisfactory. If a considerable proportion of low-melting product is to be used, it is not essential that it be wholly liquid, but only that the actual quantity of liquid present at the desired temperature be sufficient to consolidate the refractory particles with which it is mixed.

Refractoriness is a relative, rather than an absolute, term. Copper refining furnaces may be operated at 1100 and copper converters at 1250, basic brick may be burned at 1450-1550, open hearth furnaces may require 1650 and electric steel furnaces 1750°; a refractory suitable for the first two applications might be quite inadequate in refractoriness for steel production. It is therefore not possible to state categorically at what temperature low-melting products lying within the scope of this invention should form liquid, but as a general rule it may be said that the invention relates to low-melting products forming at least 50% of liquid at 1450, 75% of liquid at 1500, or wholly molten at 1550°. It also includes, regardless of the actual temperature, all systems of the type defined when the temperature of consolidation or setting of the refractory particles by means of a low-melting product is at least 220 degrees centigrade below the temperature at which liquid formation will occur when equilibrium has been established in the ultimate refractory. A large temperature difference of this kind is characteristic of the invention, and the difference will usually be substantially greater than 200 degrees.

In discussing systems involving the use of pure starting materials, one can speak with confidence as to the temperature of initial liquid formation and the degree of melting. That is not the case, however, when commercial starting materials are used, for the presence of impurities almost invariably reduces the temperature of liquid formation. Similarly, impurities may make it impossible to eliminate all liquid from the final product. It will be evident that some potential sources

of raw materials, because of their content of impurities, must be rejected altogether for application in the practice of this invention. In the practical examples which follow it will be assumed that impurities do not occur in the raw materials in sufficient quantity to affect the results to any substantial degree.

The scope of the invention is so broad, and the possible applications of the principles involved are so numerous, that the cases mentioned below are not intended to do more than provide typical examples. The invention is by no means limited in scope by the particular disclosures made herein, but only by the broad application of the principles involved in them.

If the low-melting product to be used in the consolidation of refractory particles is to be preformed, any suitable method of production may be adopted. For example, if dolomite and quartzite are to be used in the proportions required to produce a material melting below 1400°, the operation can be carried out in an electric furnace, or even in a blast furnace or cupola. The molten product issuing from the furnace may be allowed to solidify and then be crushed to the desired size, or the molten stream may be granulated by breaking it up with a jet of water, steam or air, and allowing the droplets to fall into a body of water.

If sintering rather than complete fusion is desired, a rotary kiln may be used to advantage. Such equipment, with appropriate temperature control, can be used for the production of any low-melting product, and is particularly advantageous when the product contains, at the temperature of operation, a considerable proportion of solid as well as liquid constituent. Under these conditions the product will usually issue from the kiln in the form of clinker, and can be used with or without crushing, according to its particle size.

The use of natural minerals in place of synthetic low-melting products has already been dealt with above.

#### Case 1

There is required a material for burning-in successive layers of magnesite to form the permanent bottom of an open hearth steel furnace, the object being to replace the magnesite-slag mixture so long—but rather ineffectively—used for this purpose.

One may first prepare by the fusion of serpentine, old fireclay brick and quartzite, a low-melting material containing 20%  $\text{MgO}$ , 20%  $\text{Al}_2\text{O}_3$  and 60%  $\text{SiO}_2$ . This is crushed to pass a screen of four meshes to the inch and is mixed with magnesite clinker of the same grain size in proportions of 20 to 80, and the mixture is thrown into a hot furnace. As soon as the material reaches a temperature of 1350° the low-melting product fuses and bonds the highly refractory particles together. Subsequent heat treatment of the bottom during the ordinary burning-in process brings about reaction between the constituents and consolidates the mass so that the final bottom consists of 84%  $\text{MgO}$ , 4%  $\text{Al}_2\text{O}_3$  and 12%  $\text{SiO}_2$ , in the form of periclase, spinel and forsterite. No liquid can subsequently form below 1700, and very little below 2000°. The bottom is thus burned-in even more rapidly than if slag were used, and the final bottom is of much higher refractoriness.

#### Case 2

There is required for an electric steel furnace 75 a fettling material which will set more rapidly

than burned dolomite, be resistant to slag attack, and be hard at 1750°.

Two parts of raw dolomite and one of quartz or sandstone are melted to form a slag containing 30 CaO, 21 MgO and 49% SiO<sub>2</sub>, and melting between 1350 and 1400°. This product is granulated in water, mixed with four-mesh dolomite (burned without the addition of iron oxide) in equal proportion, and the product is used for fettling. Owing to the formation of 50% liquid at 1400 and the immediate absorption of this liquid by the burned dolomite, setting is extremely rapid. The consolidated product consists exclusively of periclase and dicalcium silicate, and forms no liquid below 1980°. Since the slag consists almost exclusively of dicalcium and tricalcium silicate, with a little calcium carbide, calcium fluoride, magnesia, and other minor constituents, it has no action on the banks. (If desired, the dolomite could be used raw, but it is usually more economical to preburn it. If desired, one could also add to the final mixture a small proportion of calcium phosphate or other suitable stabilizing agent to prevent the subsequent dusting of the dicalcium silicate on cooling, but this is a refinement which does not appreciably affect the procedure or product, and does not constitute a part of the present invention.)

As to the behaviour of such a fettling material under the action of heat, it may be said that until initial fusion takes place the granular mass on the banks is soft and friable, as when originally mixed. The appearance of liquid produces in the mass a mushy condition, like that of wet snow. As the formation of refractory compounds proceeds, the mass becomes progressively harder and drier, and when the reaction is complete the consolidated material is usually very hard, with no sign of liquid. With different starting materials, the change in character of the material used for fettling varies somewhat, owing to differences in the amount and viscosity of the liquid present, the rate at which the final reactions proceed, and other factors. Frequently, however, materials of the type described will pass through all of these stages before ordinary fettling refractories show any sign of setting whatever.

#### Case 3

Difficulty is encountered in burning zirconia brick, owing to the high temperature required for the development of a bond to provide the necessary strength in the final product. Some means are required of producing a bond at a lower temperature, and at the same time of developing a stronger brick, of adequate refractoriness.

One first prepares a eutectic containing 90 BaO and 10% ZrO<sub>2</sub>, and then introduces 10% of this, as a fine constituent, into granular zirconia to be used in making brick. The molded brick are burned at 1400, a temperature easily attainable in any refractory brick kiln. At 1350 the eutectic melts, and when reaction with the zirconia and consolidation are complete a strong ceramic bond is effected, and no liquid can form below 2030°, a refractoriness which is more than adequate. In a similar way, forsterite, mullite, and other types of brick of excellent strength and high refractoriness can be made at relatively low temperatures.

#### Case 4

A rammed magnesite hearth has been installed using sodium silicate as a bond. As in the usual practice, the furnace is heated to working tem-

perature and then cooled before putting in the first charge. Cracks form, owing to thermal contraction, and steel would subsequently penetrate these, weakening the bottom and increasing its thermal conductivity. There is required a refractory material with which the cracks can be filled to prevent the penetration of steel.

Instead of preparing a highly refractory material and attempting to fill the cracks with it (which would be practically impossible) one prepares a low-melting product by sintering in a rotary kiln at a temperature of 1400 a mixture of serpentine, clay, and kyanite to make a product containing 17 MgO, 36 Al<sub>2</sub>O<sub>3</sub>, and 47% SiO<sub>2</sub>. At this temperature there is good clinkering action without complete fusion. The furnace is heated to 1500° and sufficient of the crushed sinter is then thrown into it, especially along the cracks, to fill them adequately, with some excess. The material immediately melts and runs into the cracks, where it slowly reacts with the magnesia walls to form forsterite and spinel, having melting-points of 1910 and 2135°, respectively. These refractory compounds will remain solid at the highest temperature of the furnace, and by consolidating the whole bottom, effectively prevent the penetration of steel or slag.

#### Case 5

It is desired to lower the setting temperature of one of the common thermoplastic fettling refractories which, in spite of its content of calcium ferrite and aluminate, in the absence of slag remains in a loose condition on the furnace banks until the temperature rises above 1600. It is also an objective to increase the ultimate refractoriness of this material, which is definitely plastic at 1650°.

The thermoplastic refractory contains (exclusive of its dead-burning agents, which may for the moment be regarded as impurities) approximately 72 MgO, 21 CaO and 7% SiO<sub>2</sub>. Since the lime content is approximately 60% greater than that required to form the refractory compound dicalcium silicate, the magnesia may be taken as periclase and neglected in the calculation of siliceous flux to be added; hence the system is essentially binary. There is available as a low-melting material a quantity of the mineral diopside (CaO.MgO.2SiO<sub>2</sub>). Enough of this will be added to form in the final product only dicalcium silicate from all lime and silica present. Calculation shows that the quantity required is 8.5 parts, which will be used with 91.5 parts of the thermoplastic refractory. The diopside is crushed to 20 mesh, mixed with the thermoplastic refractory, and thrown onto the banks of an open hearth furnace as a fettling material. The diopside melts at 1395°, thereby lowering the setting temperature by more than 200 degrees, and subsequently reacts with and consolidates the thermoplastic refractory to bring about a substantial increase in its refractoriness. Both of these results are important advantages. (Actually, the addition of the siliceous low-melting diopside breaks up the calcium ferrite and aluminate, and replaces them with more refractory dicalcium silicate, magnesium ferrite and magnesium aluminate (spinel), but the elimination of these fluxes is not a part of the invention.)

This procedure is in striking contrast with the practice, disclosed in the prior art, of adding a material high in lime to refractories which are to some degree thermoplastic due to the presence in them of orthosilicates of low refractoriness

(monticellite and merwinite). The new method greatly lowers the setting temperatures of the major refractory by providing a siliceous, low-melting material between the grains to be bonded, instead of actually raising the setting temperature by introducing between the plastic grains a calcareous material of high refractoriness. The consolidating reaction between the liquid low melting constituent and the highly refractory particles readily takes place under normal burning conditions.

I claim:

1. A method of consolidating refractory materials, which comprises mixing discrete particles comprising essentially refractory oxide material from a group consisting of lime, magnesia, alumina and zirconia with non-refractory material comprising essentially a low-melting compound of said oxide and being one of a group consisting of calcium silicate and calcium magnesium silicate when said oxide is lime and lime with magnesia present, magnesium silicate and magnesium aluminum silicate when said oxide is magnesia, barium zirconate when said oxide is zirconia, and aluminum silicate when said oxide is alumina, said non-refractory material becoming liquid at a temperature between 1321 and 1550° C., the mixture containing not less than 50% by weight of said discrete particles, and heating the mixture to not less than 1321° C. to melt said non-refractory material, and thus consolidate said particles into a highly refractory mass.

2. A method of consolidating refractory materials which comprises forming an intimate mixture of two types of materials, the first type being granular particles consisting essentially of refractory oxide material from a group consisting of lime, magnesia, alumina and zirconia, and the second type comprising essentially a low-melting compound of the oxide material and being one of a group consisting of calcium silicate and calcium magnesium silicate when the oxide material is lime and lime with magnesia present with the molecular ratio of lime to silica in the mixture not less than 2.0, magnesium silicate when the oxide material is magnesia with the molecular ratio of magnesia to silica in the mixture not less than 2.0, magnesium aluminum silicate when the oxide material is magnesia with a molecular ratio of magnesia to silica in the mixture not less than 2.0 and additional magnesia to alumina not less than 1.0, aluminum silicate when the oxide material is alumina with the molecular ratio of alumina to silica in the mixture not less than 1.5, and barium zirconate when the oxide material is zirconia with the molecular ratio of zirconia to baryta in the mixture not less than 1.0, and heating the mixture to not less than 1321° C. to melt said non-refractory compound and thus consolidate said particles into a highly refractory mass.

3. A method as defined in claim 1 wherein the non-refractory compound is a preformed material.

4. A method as defined in claim 1 wherein the method is carried out in a furnace lining.

5. A batch material for refractory masses and shapes, which comprises an intimate mixture of discrete particles comprising essentially refractory oxide material from a group consisting of

lime, magnesia, alumina and zirconia, and non-refractory material comprising essentially a low-melting compound of said oxide material and being one of a group consisting of (a) calcium silicate and calcium magnesium silicate when the oxide material is lime and lime with magnesia, (b) magnesium silicate and magnesium aluminum silicate when the oxide material is magnesia, (c) aluminum silicate when the oxide material is alumina, (d) barium zirconate when the oxide material is zirconia, and said mixture containing not less than 50% by weight of said discrete particles, whereby when the mixture is heated to liquefy said non-refractory material the whole mass consolidates into a product which does not melt below 1800° C.

6. A batch material for refractory masses and shapes, which comprises an intimate mixture of two types of materials, the first type being granular particles consisting essentially of refractory oxide material from a group consisting of lime, magnesia, alumina, and zirconia, and the second type consisting essentially of a low-melting compound of the refractory oxide and being one of a group consisting of (a) calcium silicate and calcium magnesium silicate when the oxide is lime and lime with magnesia present with the molecular ratio of lime to silica in the mixture not less than 2.0, (b) magnesium silicate when the oxide is magnesia with the molecular ratio in the mixture not less than 2.0, (c) magnesium aluminum silicate when the oxide is magnesia with a molecular ratio of magnesia to silica in the mixture not less than 2.0 and additional magnesia to alumina not less than 1.0, (d) aluminum silicate when the oxide is alumina with the molecular ratio of alumina to silica in the mixture not less than 1.5 and (e) barium zirconate when the oxide is zirconia and the molecular ratio of zirconia to baryta in the mixture not less than 1.0, whereby when the mixture is heated to liquefy said non-refractory material the whole mass consolidates into a product which does not melt below 1800° C.

7. A method as defined in claim 2 wherein the mixture is heated to a temperature of not less than 1550° C. to melt the non-refractory material and thus consolidate the particles into a highly refractory mass.

50

FRANK EUGENE LATHE.

#### REFERENCES CITED

The following references are of record in the file of this patent:

55

#### UNITED STATES PATENTS

| Number       | Name          | Date           |
|--------------|---------------|----------------|
| 1,300,631    | Meyer         | Apr. 15, 1919  |
| 2,015,446    | Cape et al.   | Sept. 24, 1935 |
| 60 2,089,970 | Lee           | Aug. 17, 1937  |
| 2,207,557    | Seil          | July 9, 1940   |
| 2,238,428    | Seaton et al. | Apr. 15, 1941  |

#### FOREIGN PATENTS

| Number  | Country       | Date |
|---------|---------------|------|
| 396,532 | Great Britain | 1933 |

#### OTHER REFERENCES

Glass Industry—March 1935—page 84.  
Ser. No. 342,112, Stenvik (A. P. C.), published 70 May 11, 1943.